

## UNITED STATES PATENT OFFICE

2,153,482

## LUBRICATING COMPOSITION

Carl F. Prutton, Cleveland Heights, Ohio, assignor, by mesne assignments, to The Lubri-Zol Development Corporation, Cleveland, Ohio, a corporation of Delaware

No Drawing. Application April 21, 1938,  
Serial No. 203,439

## 8 Claims.

(Cl. 87—9)

The present invention relates, as indicated, to lubrication and more particularly to a lubricating composition characterized by being capable of withstanding extreme unit pressures between the bearing surfaces which the same is called upon to lubricate, without the disadvantages of instability and gum-forming tendencies which characterize similar lubricating compositions now commonly available.

10 This application is a continuation in part of copending application Serial No. 737,070, filed July 26, 1934.

By "extreme pressures," as referred to above, is meant pressures of or in excess of 10,000 pounds per square inch, such pressures now being commonly encountered in hypoid gears, bearings, contact surfaces of cylinders and piston rings in internal combustion engines, and many other points. Such pressures tend to cause the rupture 20 of the continuous "thick film" of lubricant which separates bearing surfaces under more moderate conditions. A region of "thin-film" lubrication results which is also sometimes described as "boundary" lubrication.

25 It is a principal object of this invention, therefore to provide a method of lubricating and a lubricating composition which will operate under conditions of extreme pressure to prevent seizure between the relatively moving metallic surfaces 30 and which may be so employed without danger of deleterious effect upon the parts lubricated.

Other objects of this invention will appear as the description proceeds.

To the accomplishment of the foregoing and related ends, said invention, then, consists of the means hereinafter fully described and particularly pointed out in the claims; the following description setting forth in detail certain approved combinations of ingredients embodying my invention, such disclosed means constituting, however, but certain of various forms in which the principle of the invention may be used.

Broadly stated, this invention comprises a method of lubricating and a lubricating composition wherein a minor proportion of a halogen-bearing dibenzyl disulphide is employed in conjunction with a hydrocarbon oil.

While for certain specialized uses the halogen-bearing dibenzyl disulphide may be employed as the sole lubricant this invention contemplates that in general it will be employed as an addition agent to mineral lubricating oils in amounts ranging from about .2% to about 20% by weight, based on the amount of mineral oil. For most purposes and under most conditions from about 1%

to about 5% of the addition agent will be found to be sufficient to accomplish the end desired although for certain uses and conditions amounts up to 10% and even 20% are occasionally preferred. The final product should contain at least 2% of the addition agent in order that it may exhibit sufficient extreme pressure properties to be commercially feasible.

While the oil base is referred to above as a mineral lubricating oil, it is to be understood that 10 any other suitable hydrocarbon lubricating oil, whether naturally occurring or synthetic, may be employed as the oil base.

It is also within the contemplation of this invention to provide the addition agent in the form 15 of a concentrate in a suitable oil, said oil containing rather large percentages of the addition agent. Such concentrates are employed for future blending with a lubricating oil in the proportions desired for the particular conditions of 20 use.

It is believed that under conditions of extreme pressure the addition agent reacts chemically or physico-chemically with the metallic surfaces to form a non-fluxing surface which will not seize 25 or score. This invention is not intended to be limited, however, by any particular theory or explanation of the action upon the metallic surfaces.

All of the various halogens are effective when 30 employed in accordance with the present invention but chlorine is generally preferred inasmuch as it is the least expensive and one of the most effective of the halogens. Bromine and fluorine are more expensive and the latter is relatively difficult to handle but they are each usable in accordance with this invention. Iodine is not so readily obtainable as the other halogens and is quite expensive but it also is satisfactory in providing effective addition agents. It should also 40 be noted that two or more different halogens may be present in the same molecule. The brom-chlor and fluorinated chlorine or bromine compounds give especially satisfactory results.

When a chlorine-bearing dibenzyl disulphide is 45 employed as the addition agent, it will preferably contain from about 10% to about 60% chlorine although both larger and smaller percentages may occasionally be preferred.

Halogen-bearing dibenzyl disulphide is a particularly satisfactory addition agent to mineral oils because, in addition to its effectiveness, it is relatively chemically inactive at ordinary temperatures and under ordinary pressures but under 50 conditions of extreme pressure it will react with 55

the relatively moving metallic surfaces to form an anti-fluxing film and prevent seizure and scoring of said surfaces.

The halogen not only aids in rendering the final composition more effective to resist high pressures but also greatly increases the solubility of the addition agent in mineral oils.

Of the halogen-bearing dibenzyl disulphides, di (chlor-benzyl) disulphide, disclosed in co-pending application Serial Number 737,070, has proven particularly effective and satisfactory. This compound may be prepared in the manner described in my co-pending application Serial Number 193,960, filed March 4, 1938.

When still greater resistance to extreme pressure conditions is desired than that afforded by the addition agent of this invention alone it may often be found advantageous to employ a small amount of a separate organic halogen compound which will cooperate with the addition agent of this invention to increase the film strength of the lubricant (as indicated on the Almen machine) to a degree greater than the sum of the effects of either addition agent when used alone.

While the lubricating compositions which have been described herein as illustrating one embodiment of the invention have been generally referred to as "oils," i. e., liquids, this invention is, however, also especially applicable to the solid and semi-solid types of lubricants commonly referred to in the trade as greases, bodied oils, etc., and which may contain soaps such as sodium, calcium, lead, and aluminum naphthenates, stearates, and oleates.

The following table shows the results obtained when testing various percentages of chlor-dibenzyl disulphide in an SAE 160 lubricating oil on the Almen machine:—

| Percent chlor-dibenzyl disulphide | Almen (pounds) |
|-----------------------------------|----------------|
| .5                                | 19             |
| 1.0                               | 20             |
| 1.5                               | 21             |
| 2.25                              | 22             |

On a modification of the Faville-Levalley machine employing a flat block the following results were obtained:—

| Percent chlor-dibenzyl disulphide | Faville-Levalley dial reading |
|-----------------------------------|-------------------------------|
| 2                                 | 3000                          |
| 3                                 | 2125                          |
| 2+1% dibenzyl disulphide          | 2375                          |
| Plain oil (SAE 160)               | 750                           |

The two tables above given clearly show the effectiveness of even small percentages of the addition agent.

While mineral oil generally is the principal ingredient of the lubricant, it is not essential that it be the only ingredient other than the addition agent, provided that there be no additional ingredient which is incompatible with such addition agent. It is within the contemplation of this invention to include, if necessary or desirable, such other addition agents as are commonly added to improve the viscosity index or cold test of the lu-

bricant and a lubricating composition according to this invention which also has a separate oiliness increasing agent has been found to be especially effective.

explained, change being made as regards the 5

The terms "halogen-bearing" and "chlorine-bearing" as employed in the appended claims is obviously intended to mean halogen, or more specifically chlorine, in chemical combination.

Other modes of applying the principle of my 10 invention may be employed instead of the one composition and method disclosed, provided the ingredients or steps stated by any of the following claims or the equivalent of such stated ingredients or steps be employed.

I therefore particularly point out and distinctly claim as my invention:—

1. An extreme pressure lubricating composition comprising a major proportion of lubricating oil 20 the film strength of which has been substantially increased by the inclusion therein of a minor proportion of a halogen-bearing dibenzyl disulphide.

2. An extreme pressure lubricating composition comprising a major proportion of lubricating oil 25 the film strength of which has been substantially increased by the inclusion therein of from an effective amount to 20% of a halogen-bearing dibenzyl disulphide.

3. An extreme pressure lubricating composition 30 comprising a major proportion of lubricating oil the film strength of which has been substantially increased by the inclusion therein of from about .2% to about 10% of a halogen-bearing dibenzyl disulphide.

4. An extreme pressure lubricating composition comprising a major proportion of lubricating oil the film strength of which has been substantially increased by the inclusion therein of from about 1% to about 5% of a halogen-bearing dibenzyl 40 disulphide.

5. An extreme pressure lubricating composition comprising a major proportion of lubricating oil the film strength of which has been substantially increased by the inclusion therein of a minor 45 proportion of a chlorine-bearing dibenzyl disulphide.

6. An extreme pressure lubricating composition comprising a major proportion of lubricating oil the film strength of which has been substantially 50 increased by the inclusion therein of from an effective amount to 20% of a chlorine-bearing dibenzyl disulphide.

7. An extreme pressure lubricating composition comprising a major proportion of lubricating oil the film strength of which has been substantially 55 increased by the inclusion therein of from about .2% to about 10% of a chlorine-bearing dibenzyl disulphide.

8. An extreme pressure lubricating composition comprising a major proportion of lubricating oil the film strength of which has been substantially increased by the inclusion therein of from about 1% to about 5% of a chlorine-bearing dibenzyl 60 disulphide.

CARL F. PRUTTON.

CERTIFICATE OF CORRECTION.

Patent No. 2,153,482.

April 4, 1939.

CARL F. PRUTTON.

It is hereby certified that error appears in the printed specification of the above numbered patent requiring correction as follows: Page 2, second column, line 5, strike out the words "explained, change being made as regards the" and insert the same after the word "one" in line 11; and that the said Letters Patent should be read with this correction therein that the same may conform to the record of the case in the Patent Office.

Signed and sealed this 23rd day of May, A. D. 1939.

Henry Van Arsdale

(Seal)

Acting Commissioner of Patents.